

Oct. 20, 1936.

C. A. BRAUCHLER

2,057,669

METHOD OF FORGING GEAR BLANKS

Filed July 2, 1934

2 Sheets-Sheet 1



Fig. 2

Fig. 1



Fig. 3



Fig. 4



Fig. 5

INVENTOR  
C.A.Brauchler  
BY  
Grease and Bishop  
ATTORNEYS

Oct. 20, 1936.

C. A. BRAUCHLER

2,057,669

METHOD OF FORGING GEAR BLANKS

Filed July 2, 1934

2 Sheets-Sheet 2



Fig. 6



INVENTOR

C. A. Brauchler  
BY  
Freese and Bishop  
ATTORNEYS

Fig. 7

## UNITED STATES PATENT OFFICE

2,057,669

## METHOD OF FORGING GEAR BLANKS

Charles A. Brauchler, Canton, Ohio

Application July 2, 1934, Serial No. 733,471

8 Claims. (Cl. 29—159.2)

The invention relates to the forging of gear blanks and the like and more particularly to a method of precision forging such parts so accurately that no machine work is required upon 5 the gear blanks excepting the cutting of the gear teeth.

Under present practice forged gear blanks and the like are produced in dies having considerable draft which is necessary in order that the forgings will not stick or bind in the dies in which they are formed. This draft in the dies produces a considerable peripheral taper from the center toward both sides of the forged gear blank as well as a considerable oppositely disposed flare in the 15 center opening of the forged gear blank. This necessitates machining of the peripheral portion as well as of the central opening in the gear blank before the blank is in condition for cutting of the gear teeth thereon.

20 The present improvement contemplates the production of precision forgings for gear blanks and the like which eliminates this peripheral taper as well as the flaring of the center opening of the forged blank, thus eliminating machining 25 of either the outside or inside of the forged gear blank.

The objects of the improvement may be accomplished by first forging the gear blank or the like with the usual draft or taper at the periphery 30 and within the center opening thereof, the top and bottom sides of the forging being flared or inclined toward the periphery and the central opening, producing an excess of metal at these points. The flash and web are then sheared in 35 the usual manner and the hot forging thus produced is placed in a press equipped with dies shaped to produce the desired finished form of gear blank, and therein pressed to the desired shape, the excess metal at these high points of 40 the forging being displaced so as to produce a precision forged gear blank having straight sides around its periphery and center opening.

An embodiment of the invention is illustrated in the accompanying drawings, in which

45 Figure 1 is an elevation of a bar blank from which a forged gear blank or the like may be produced;

Fig. 2, an elevation of the blank after it has been hammered to the proper shape for placing in 50 the forging dies;

Fig. 3, a transverse sectional view through the partly completed forging as it emerges from the forging dies;

55 Fig. 4, a similar view after the flash and web have been sheared from the forging; and

Fig. 5, a transverse sectional view through the improved precision forging produced by the method to which the invention pertains;

Fig. 6, a sectional elevation of a portion of the press and dies in which the final operation is performed showing the partly completed product as 5 illustrated in Fig. 4 in position in the lower die of the press; and

Fig. 7, an enlarged sectional view of the dies shown in Fig. 6 shown in the closed or operative 10 position showing a completed precision forging therein.

Similar numerals refer to similar parts throughout the drawings.

In carrying out the invention a cylindric bar 15 blank as indicated at 10 in Fig. 1 is heated to a forging temperature and is then given one or two blows by a drop hammer to flatten the same to substantially the shape shown at 10a in Fig. 2.

The still hot blank 10a is then placed in the 20 dies of a drop hammer which are shaped to produce the partly finished forging shown in Fig. 3. These dies have the usual draft producing the oppositely disposed tapers 11 around the periphery of the forging while the center opening 12 25 thereof is oppositely flared as shown at 13.

The dies used for this purpose are so shaped as to form an annular concavity 14 in the upper face of the forging, producing the high points 15 and 16 adjacent to the periphery and the center opening respectively. In like manner the lower die forms high points 17 and 18 on the lower side of the forging adjacent to the periphery and central opening respectively.

The usual flash 19 and web 20 are formed in 35 the forging operation and while the forging is still hot, this flash and web are sheared in the usual manner, the partly completed product as shown in Fig. 4 being then placed in the lower die 21 of a press as shown in Fig. 6.

The bed 22 of this press is provided with the fixed stem or plunger 23 of cylindric form which is located through an opening 24 in the lower die block 25, whereby the die block may be slidably moved in vertical direction upon the plunger. The lower die block 25 is suspended from the head 26 of the press as by the bolts 27 upon which the die block may slidably move vertically as will be later described.

The upper die impression 28 is formed in the 50 movable head 26 of the press, having straight side walls to form the periphery of the gear blank straight and is provided with the central opening 29 to receive the plunger 23 when the head is moved downward to close the dies upon 55

the partly completed product, as shown in Fig. 7, pressing the hot forging into the shape shown at 30 in Figs. 5 and 7, the excess metal at the high points 15 and 17 being forced outward 5 against the side walls of the upper die 28, producing the straight peripheral wall 31, while the excess metal at the high points 16 and 18 is forced inward against the plunger, producing the straight walls 32 of the central opening. 10 10 In like manner, as this excess metal is displaced, the flat upper surface 33 and flat lower surfaces 34 and 35 are formed upon the gear blank. The forging thus produced is accurate as to shape and size and needs no machining 15 excepting the necessary cutting of the gear teeth in the peripheral portion thereof.

As the head 26 of the press is again raised, the dies will be separated leaving the finished forging upon the lower die and tightly surrounding 20 the plunger 23 due to contraction of the cooling metal in the forging. As the head reaches the upper limit of its movement, as shown in Fig. 6, the die block 25 will be raised to the top of the plunger 23, sliding the forging 25 upward off of said plunger so that it may be easily removed from the lower die.

It has been found in practice that the improved method of forging gear blanks and the like compensates for any inaccuracy or unevenness 30 in the partly finished product as shown in Figs. 3 and 4, which may be due to wear in the dies for forming the same, since the plunger 23 cooperating with the dies in the press, as shown in Figs. 6 and 7, accurately centers the 35 forging within the dies.

I claim:

1. The method of producing forged metal gear blanks and the like which comprises forging a metal article having tapered side walls with an 40 adjoining concaved face producing an excess of metal at the intersection of said side walls and said adjoining face and then subjecting said article while heated to pressure causing said excess metal to flow into the side walls.

45 2. The method of producing forged metal gear blanks and the like which comprises forging a metal article having tapered side walls with an adjoining face flared toward said side walls producing an excess of metal at the intersection 50 of said side walls with said adjoining face and then subjecting said article while heated to pressure causing the metal in said flared portion to flow into the side walls.

3. The method of producing forged metal gear 55 blanks and the like which comprises forging a metal article having tapered side walls and a flared opening with an adjoining concaved face producing an excess of metal at the intersections of the concaved face with the side walls and with

said flared opening and then subjecting said article while heated to pressure flattening said concaved face and causing the excess metal therefrom to flow into the side walls and the walls of said opening. 5

4. The method of producing a forged gear blank and the like which comprises forging an article with oppositely tapered side walls and an oppositely flared central opening, the top and bottom faces thereof having an excess of 10 metal adjacent to the periphery and adjacent to the central opening, and then subjecting said article while heated to pressure causing said excess metal to flow into the side walls and the walls of the central opening. 15

5. The method of producing forged metal gear blanks and the like which comprises forging an article with oppositely tapered peripheral walls, the top and bottom faces thereof being concaved producing an excess of metal adjacent 20 to the periphery of said articles, and then subjecting said article while heated to pressure causing said excess metal to flow into the side walls.

6. The method of producing forged metal 25 gear blanks and the like which comprises forging a metal article having a flared opening, the face adjacent to the larger end of the opening being concaved producing an excess of metal surrounding the opening, and then subjecting 30 said article while heated to pressure causing said excess metal to flow into the walls of the opening.

7. The method of producing forged metal gear blanks and the like which comprises forging a 35 metal article having oppositely tapered side walls and adjoining faces flared toward the side walls producing an excess of metal at the intersection of said side walls and said adjoining faces and then subjecting the article while heated to 40 pressure causing said excess metal to flow into the side walls to produce straight side walls and flat adjoining faces. 45

8. The method of producing forged metal gear blanks and the like which comprises forging a 50 metal article having oppositely tapered side walls and an oppositely flared central opening and adjoining faces flared toward said side walls and toward said central opening producing an excess of metal at the intersections of said adjoining faces with the side walls and with the central opening, and then subjecting the article while heated to pressure causing said excess of metal to flow into the side walls and central opening to produce straight side walls 55 and a straight central opening and flat adjoining faces.

CHARLES A. BRAUCHLER.